

June 22, 1948.

W. T. HANSON, JR., ET AL  
PROCESS OF PRODUCING MULTICOLOR PHOTOGRAPHIC  
IMAGES IN A SINGLE EMULSION LAYER

2,443,909

Filed June 28, 1946



Wesley T. Hanson Jr.  
Thomas H. Farrell  
INVENTORS

BY *Newton M. Perrins*  
*R. Frank Smith*  
ATTORNEYS

## UNITED STATES PATENT OFFICE

2,443,909

PROCESS OF PRODUCING MULTICOLOR  
PHOTOGRAPHIC IMAGES IN A SINGLE  
EMULSION LAYERWesley T. Hanson, Jr., and Thomas H. Farrell,  
Rochester, N. Y., assignors to Eastman Kodak  
Company, Rochester, N. Y., a corporation of  
New Jersey

Application June 28, 1946, Serial No. 679,890

3 Claims. (Cl. 95—2)

1

The present invention relates to color photography and particularly to a method for forming multi-color images in a single photographic emulsion layer.

The formation of multi-color images by color development in a multi-layer photographic material is well known and it has also been proposed to form images of a single color in a single emulsion layer by color development. The formation of multi-color images in a single emulsion layer by color development has also been suggested but such methods have generally not been successful unless the color-forming or coupling components are incorporated in the emulsion layer, as in the "mixed grain" methods.

It is therefore an object of the present invention to provide a method for the formation of multi-color images in a single silver halide emulsion layer by color development. Other objects will appear from the following description of our invention.

These objects are accomplished according to the method more fully described hereinafter, an essential feature of which is the successive exposure of the emulsion layer to color separation images followed by development of the residual silver halide in a color developer forming a soluble dye and rehalogenization of all of the developed silver.

The accompanying drawing is a series of sectional views of film at various stages in the process according to our invention.

As stated above, our method enables the formation of a multi-color photographic image, for example, an image in three colors, in a normal silver halide emulsion layer. This layer is successively exposed to light under the images which are to be recorded and if a natural color image is to be formed, it is customary to use color separation negatives for this purpose. The negatives are registered in some suitable way and after each exposure, the film is developed in a color-forming developer suitable for the formation of an image representing the particular color separation negative to which the film has been exposed. After each exposure step except the last, the film is developed in a color-forming developer followed by a flash exposure and development in a color-forming developer which produces a soluble dye image. The soluble dye is washed from the layer and the silver images are then rehalogenized and, if necessary, resensitized before the next exposure. After the last exposure to a color separation negative, the silver images are removed in the usual way. This

2

process will be more readily understood by reference to the following description of a method of forming a natural-color picture in an emulsion layer.

5 A film having a normal positive silver halide emulsion is treated according to the following procedure:

- (1) Expose through a red separation negative.
- (2) Develop for 6 minutes in a solution of the

10 following composition which forms a cyan image:

|                                              | Grams |
|----------------------------------------------|-------|
| 2-amino-5-diethylamino toluene hydrochloride | 2.5   |
| 15 Sodium sulfite                            | 20    |
| Sodium carbonate                             | 20    |
| Potassium bromide                            | 2     |
| 6-nitro-benzimidazole                        | .03   |
| Sodium thiocyanate                           | .5    |
| Sodium hydroxide                             | .5    |
| 20 2,4-dichloro- $\alpha$ -naphthol          | 1     |
| Water to 1 liter                             |       |

- (3) Wash 3 minutes in water.

25 (4) Flash exposure sufficiently to totally expose residual silver halide.

(5) Develop 8 minutes in the following solution which forms a soluble dye image:

|                                                 | Grams |
|-------------------------------------------------|-------|
| 30 2-amino-5-diethylamino toluene hydrochloride | 2.5   |
| Sodium sulfite                                  | 20    |
| Sodium carbonate                                | 20    |
| Potassium bromide                               | 0.5   |
| 6-nitro-benzimidazole                           | .01   |
| 35 Sodium thiocyanate                           | .5    |
| Sodium hydroxide                                | .5    |
| Resorcinol                                      | .5    |
| Water to 1 liter                                |       |

- 40 (6) Wash 3 minutes in water.

(7) Treat for 6 minutes in the following solution which converts all silver to silver bromide:

5 grams per liter of potassium dichromate

40 grams per liter of potassium alum and

45 20 grams per liter of potassium bromide in a solution adjusted with sulfuric acid to a pH of 2.7 to 2.8.

- (8) Wash 6 minutes in water.

50 (9) Resensitize by treating the film for two minutes in a solution containing 5 grams per liter of sodium bisulfite.

- (10) Wash 3 minutes with water.

- (11) Dry (or this step may be omitted).

- (12) Register and expose film through green 55 separation negative.

(13) Develop 6 minutes in the following solution which produces a magenta image:

|                                              | Grams |
|----------------------------------------------|-------|
| 2-amino-5-diethylamino toluene hydrochloride | 2.5   |
| Sodium sulfite                               | 20    |
| Sodium carbonate                             | 20    |
| Potassium bromide                            | 2.    |
| 6-nitro-benzimidazole                        | .03   |
| Sodium thiocyanate                           | .5    |
| Sodium hydroxide                             | .5    |
| 1-phenyl-3-methyl-5-pyrazolone               | 3     |
| Elon                                         | 0.1   |
| Water to 1 liter                             |       |

Repeat steps 3 through 11.

(14) Register and expose through blue separation negative.

(15) Develop for 9 minutes in the following solution which produces a yellow image:

|                                              | Grams |
|----------------------------------------------|-------|
| 2-amino-5-diethylamino toluene hydrochloride | 2.5   |
| Sodium sulfite                               | 20    |
| Sodium carbonate                             | 20    |
| Potassium bromide                            | 2     |
| 6-nitro-benzimidazole                        | 0.12  |
| Sodium thiocyanate                           | .5    |
| Sodium hydroxide                             | 2.5   |
| o-Benzoyl acet-anilide                       | 4     |
| Water to 1 liter.                            |       |

(16) Bleach the silver image in the following solution:

|                        | Grams |
|------------------------|-------|
| Potassium ferricyanide | 10    |
| Potassium bromide      | 5     |
| Water to 250 cc.       |       |

(17) Fix in a 30% solution of hypo.

(18) Wash.

(19) Dry.

One of the important features of our process is the use of a color developer for complete development of the non-image-forming grains. This developer, composed of the same developing agent as the color developer and of resorcinol as a coupler, forms a water-soluble dye image and develops the non-image residual silver halide to the same state as the image-forming color developer so that after rehalogenizing, the film is composed of a dye image plus a rehalogenized emulsion of uniform sensitivity characteristics. Omission of this developer leaves the grains which were used in forming the first color image in a very different state from the residual grains so that the successive exposures to the other separation images are not independent of the first image present, as they should be.

The coupling agents used to form the colored images may be any of the well known coupling agents such as those described in U. S. Patents 2,039,730, 2,313,586, 2,362,598, reissue 22,329, 1,969,479, 2,343,703, 2,108,602, 2,271,238 and 2,364,675. The developing agents may be any of those well known in the color development art and the same developing agent need not be used for both the image-forming development and the development of the soluble dye. It is preferable however, that these developing agents be similar so that the silver images produced in different parts of the layer are similar.

In place of resorcinol, other couplers capable of forming soluble dye images may be used such as 1,3-dihydroxy-4-chlorobenzene, 2,4 - dihydroxy

benzoic acid, phloroglucinol salicylactic acid, resacetophenone, o-phenol sulfonic acid, 1-naphthol-5-sulfonic acid, 2-naphthol-6-sulfonic acid, 1-amino-8-naphthol-4-sulfonic acid, 1-amino-8-naphthol-3,6-disulfonic acid, 1,8-dihydroxynaphthalene-3,6-disulfonic acid, 2-amino-8-naphthol-6-sulfonic acid, 1-phenyl-5-pyrazolone-3-carboxylic acid, 1-p-sulfophenyl-3-methyl-5-pyrazolone, 1-p-sulfophenyl - 5 - pyrazolone - 3 - carboxylic acid, 3,5-diaminobenzoic acid, 1,3,5-triaminobenzene, 2,4,6-triaminobenzoic acid, 2,4,6-triaminochlorobenzene, diethylmalonate, barbituric acid, etc.

Our invention will be further illustrated by reference to the accompanying drawing.

A sensitive photographic element comprising a support having thereon a silver halide emulsion layer 10 as shown in step 1 of the drawing is exposed through a red separation negative image and developed in a developing solution which produces a cyan image 11 in emulsion layer 10 as shown in step 2 of the drawing and leaves undeveloped silver halide in the unexposed portions of the emulsion layer. The film is then flashed to fully expose the residual silver halide and color developed in a solution containing resorcinol or other coupler which produces a soluble dye image and metallic silver 12 as shown in step 3 of the drawing. The silver image in the region of the cyan dye image 11 and the silver image 12 are then converted to silver halide 13 as shown in step 4 of the drawing. Since both regions of the layer have been developed in a color-forming developer and reconverted to silver halide in the same bath, the silver halide in the entire emulsion layer is now uniformly light-sensitive.

The emulsion layer is then exposed through a green separation negative image in register with the first exposure and the emulsion layer is developed in a color-forming developer which produces a magenta image 14 in the emulsion layer. The image 14 may coincide partially or completely with the cyan image or may be in a separate region of the emulsion layer. It is entirely independent of the cyan image previously formed in the layer.

The emulsion layer is again flashed with light which uniformly exposes the residual silver halide and again color developed in a color developer containing resorcinol or other coupler which produces a soluble dye image in the residual halide of the emulsion layer and metallic silver 15 as shown in step 6 of the drawing. The silver is again converted to silver halide as shown as 16 in step 7 of the drawing and is thereby rendered uniformly light-sensitive as before.

The emulsion layer is then exposed through the blue separation negative image in register with the cyan and magenta images previously formed in the layer and developed in a yellow color-forming developer to form the yellow image 17 as shown in step 8 of the drawing. The silver images are then removed leaving the cyan, magenta and yellow images 11, 14 and 17 in the emulsion layer.

It will be understood that the examples and modifications described herein are illustrative only and that our invention is to be taken as limited only by the scope of the appended claims.

We claim:

1. The process of color photography which comprises exposing a silver halide emulsion layer to a color component image, developing the layer in a color-forming developer which forms a silver

and insoluble dye image, uniformly exposing said layer and developing all residual silver halide in a color-forming developer of substantially the same composition and containing the same developing agent as said first-mentioned developer, which forms a silver and soluble dye image, washing the soluble dye from the layer, rehalogenizing all developed silver to silver halide, and repeating the steps of exposure to a color component image and development in a color-forming developer forming an insoluble dye image with at least one other color component image, and removing all developed silver images from the layer.

2. The process of color photography which comprises exposing a silver halide emulsion layer to a color component image, developing the layer in a color-forming developer which forms a silver and insoluble cyan dye image, uniformly exposing said layer and developing all residual silver halide in a color-forming developer of substantially the same composition and containing the same developing agent as said first-mentioned developer, which forms a silver and soluble dye image, washing the soluble dye from the layer, rehalogenizing all developed silver to silver halide, exposing the layer to a second color component image in register with the first image, developing the layer in a color-forming developer which forms silver and insoluble magenta dye image, uniformly exposing said layer and developing all residual silver halide in a color-forming developer of substantially the same composition and containing the same developing agent as said first-mentioned developer, which forms a silver and soluble dye image, washing the soluble dye from the layer, rehalogenizing all developed silver to silver halide, exposing the emulsion layer to a third color component image, developing the layer in a color-forming developer which forms a silver and insoluble yellow dye image, and removing all developed silver images from the layer.

3. The process of color photography which comprises exposing a silver halide emulsion layer to a red color component image, developing the layer in a color-forming developer which forms a silver and insoluble cyan dye image, uniformly exposing said layer and developing all residual silver halide in a color-forming developer which contains resorcinol as a coupler which has substantially the same composition and contains 5 the same developing agent as said first-mentioned developer, and which forms a silver and soluble dye image, washing the soluble dye from the layer, rehalogenizing all developed silver to silver halide, exposing the layer to a green color 10 component image, developing the layer in a color-forming developer which forms a silver and insoluble magenta dye image, uniformly exposing said layer and developing all residual silver halide in a color-forming developer which contains 15 resorcinol as a coupler which has substantially the same composition and contains the same developing agent as said first-mentioned developer, and which forms a silver and soluble dye image, washing the soluble dye from the layer, rehalogenizing all developed silver to silver halide, exposing the layer to a blue color component image, developing the layer in a color-forming developer which forms a silver and insoluble yellow dye image and removing all developed silver 20 images from the layer.

WESLEY T. HANSON, JR.  
THOMAS H. FARRELL.

## REFERENCES CITED

- 35 The following references are of record in the file of this patent:

## UNITED STATES PATENTS

| Number       | Name          | Date          |
|--------------|---------------|---------------|
| 40 1,976,301 | Seymour et al | Oct. 9, 1934  |
| 2,210,905    | Eggert et al. | Aug. 13, 1940 |
| 2,244,589    | Yanket        | June 3, 1941  |
| 2,336,243    | Hauson        | Dec. 7, 1943  |